

# UNITED STATES PATENT OFFICE.

FRANK PERRY, OF TIPTON, ENGLAND, ASSIGNOR TO METALLOIDS LIMITED, OF TIPTON, ENGLAND.

## SCALING AND ANNEALING OF METAL ARTICLES.

1,261,606.

Specification of Letters Patent.

Patented Apr. 2, 1918.

No Drawing.

Application filed February 15, 1917. Serial No. 148,873.

*To all whom it may concern:*

Be it known that I, FRANK PERRY, a subject of the King of Great Britain and Ireland, residing at Tibbington Works, Tipton, in the county of Stafford, England, have invented certain new and useful Improvements Relating to the Scaling and Annealing of Metal Articles, of which the following is a specification.

10 This invention relates to the treatment of Mond or other producer or like gas for use in annealing metal articles or reducing or preventing the formation of non-metallic surfaces such as coatings of oxid on such articles when subjected to the heat of a muffle or the like.

15 In processes previously proposed various constituents have been removed from the reducing gas, such as water vapor, sulfur compounds and unsaturated hydrocarbons, but none of these has been entirely effective in preventing the formation of film like deposits of non-metallic substances on the surfaces of the articles while in the chamber.

20 The present invention consists in removing the saturated hydrocarbons such as methane in addition to such deleterious constituents as excess water vapor, sulfur compounds and unsaturated hydrocarbons all 25 these constituents being removed before the gas enters the muffle.

25 In one convenient manner of carrying the invention into effect, the gas before it enters the muffle and after it has been treated for the removal of water vapor, sulfur compounds and unsaturated hydrocarbons if these are present, is passed through a hot chamber containing loose pieces of iron, or through a hot iron tube, the iron serving to 30 combine with and consequently remove those constituents which are harmful to the iron or other metal articles to be treated. I find the most advantageous temperature for the iron is about 250° C., and I operate, 35 therefore, at or near this temperature. If the iron is excessively heated it no longer removes the methane. Passing producer gas through an iron tube for the removal of

sulfur compounds has been proposed, but the temperature necessary is too high to 50 make the removal of methane or other saturated hydrocarbons possible.

Periodically when the iron becomes coated with deposits from the gas it is replaced by fresh material. 55

By this invention perfectly clean metal surfaces can be produced or preserved in annealing operations in a simple and inexpensive manner.

The invention is not limited to any particular means for removing the saturated hydrocarbons, and the removal of the other constituents forms *per se* no part of the invention. 60

Having thus described my invention what 65 I claim as new and desire to secure by Letters Patent is:—

1. A process of annealing metal articles, which consists in introducing into the oven containing the articles, Mond gas purified 70 by removing the saturated hydrocarbons such as methane in addition to such deleterious constituents as excess water vapor, sulfur compounds, and unsaturated hydrocarbons. 75

2. A process of annealing metal articles, which consists in introducing into the muffle containing the articles, Mond gas first purified by removing therefrom sulfur compounds, water vapor and unsaturated hydrocarbons and passing such purified gas prior to its entrance to the muffle containing the metal articles over iron at a temperature about 250° C., substantially as described. 80

3. A process of annealing metal articles 85 which consists in introducing into the muffle containing the articles, Mond gas first purified by removing therefrom sulfur compounds, water vapor and unsaturated, hydrocarbons and then passing the purified gas 90 through an iron tube at a temperature of about 250° C., prior to entrance to the muffle, substantially as described.

In testimony whereof I have signed my name to this specification.

FRANK PERRY.